

## UNITED STATES PATENT OFFICE

2,343,789

IMPROVING QUALITY OF OXIDIZED  
ASPHALTSKenneth G. Morris, Westfield, N. J., assignor to  
Standard Oil Development Company, a corpora-  
tion of DelawareNo Drawing. Application January 8, 1941,  
Serial No. 373,613

3 Claims. (Cl. 196—74)

This invention relates to improvements in the manufacture of oxidized coating asphalts and it relates particularly to improvement in the softening point-penetration relationship of oxidized asphalts.

In the preparation of coating asphalts by the oxidation of asphalt fluxes, difficulties have been encountered in producing satisfactory coating asphalt from straight reduced petroleum oil fluxes. This is the result of the demand for asphalt having rather narrow limits in softening point-penetration relationship in combination with low stain. This softening point-penetration relationship of an oxidized asphalt can generally be improved by using a softer oxidizing base, but this also raises stain or causes some other physical property to become unsuitable. A typical asphalt suitable for use in the manufacture of asphalt roofing materials may have the following properties: A maximum stain of 3½ and penetration at 77° F./100 grams/5 secs. of 18 to 22 for 218—222° softening point asphalts.

The stain referred to in this case is obtained by a method which consists briefly of placing a button of coating asphalt between several thicknesses of paper under a dead weight of 400 grams, and maintaining the assembly at a controlled temperature of 130° F. for five days to insure contact of the asphalt and papers. The degree of staining is indicated by the number of sheets of paper on each side through which the "oils" in the asphalt penetrate.

Many crudes when straight reduced by distillation yield asphalt fluxes which do not oxidize to coating asphalts meeting the requirements given above as typical specifications. However, according to this invention, oxidizing bases can be prepared which will oxidize to satisfactory asphalt by eliminating the "heart" or heavy cut

from a reduced crude by distillation or other suitable means and blending the high softening point asphalt bottoms with a suitable light oil to the desired flux consistency. For example, a

5 Venezuelan crude was first topped by distilling off 25% of the volatile fractions, such as gasoline and kerosene. The reduced crude was then distilled to give 43% of 187° F. softening point bottoms, 21% of a heavy side stream (heart) cut 10 having a flash of 585° F. and 36% of a 385° F. flash point, light overhead distillate. The 187° F. high softening point bottoms was blended with the 385° F. flash temperature light overhead distillate to give various grades of asphalt fluxes, 15 and similar consistency bases were also prepared by blending the high softening point asphalt with a 485° F. flash point oil cut prepared by topping the 385° F. flash overhead distillate.

The 75% reduced Venezuelan crude was also 20 reduced by distillation (that is, straight reduction) to 74°, 84° and 102° F. softening point asphalt fluxes, which were then oxidized to coating asphalts. The data table summarizing physical properties of coating asphalts oxidized from both straight reduced and blended fluxes shows 25 that the consistency of the blended flux as well as properties of the light distillate used control the improvement obtained. The coating asphalts oxidized from 76° F. and 84° F. softening point blended fluxes made with 385° F. flash distillate have the desirable combination of properties previously mentioned, which are not obtainable by oxidation from straight reduced fluxes of the 30 same consistency. The results on the blends made with the 485° F. flash overhead likewise show that satisfactory coating asphalts will only result from the use of overhead within a limited 35 flash or consistency range.

## OXIDATION STUDIES

Comparison of coating asphalts oxidized from straight reduced and blends of bottoms and overhead fractions from reduced Venezuelan crudes

|                                    | 75° softening point |          |         | 85° softening point |          |         | 180/200 penetration |          |         |
|------------------------------------|---------------------|----------|---------|---------------------|----------|---------|---------------------|----------|---------|
|                                    | Regular             | Straight | Reduced | Regular             | Straight | Reduced | Regular             | Straight | Reduced |
| 1. Oxidizing base:                 |                     |          |         |                     |          |         |                     |          |         |
| Composition—                       |                     |          |         |                     |          |         |                     |          |         |
| Per cent 187° F. S. P. btrms       | 62                  | 53       | 47      | 66                  | 58       | 42      | 73.5                | 63       | 37      |
| Per cent 385° flash O. H.          | 38                  |          |         | 34                  |          |         | 26.5                |          |         |
| Per cent 485° flash O. H.          |                     |          |         |                     |          |         |                     |          |         |
| Physical inspections—              |                     |          |         |                     |          |         |                     |          |         |
| Spec. grav. at 60° F.              | 1.004               | 1.015    | 1.015   | 1.010               | 1.011    | 1.013   | 1.015               | 1.020    | 1.020   |
| Flash, ° F.                        | 485                 | 415      | 505     | 500                 | 420      | 515     | 505                 | 420      | 525     |
| Softening point, ° F.              | 74                  | 76       | 78      | 84                  | 84       | 87      | 102                 | 104      | 107     |
| Pen. 77°/100 g./5"                 | 300+                | 300+     |         | 300+                | 300+     |         | 176                 | 188      | 162     |
| Pen. 32°/200 g./60"                | 216                 | 290      | 162     | 121                 | 168      | 107     | 32                  | 58       | 46      |
| 2. 215/225° S. P. coating asphalt: |                     |          |         |                     |          |         |                     |          |         |
| Physical inspections—              |                     |          |         |                     |          |         |                     |          |         |
| Spec. grav. at 60° F.              | 1.031               | 1.031    | 1.032   | 1.031               | 1.032    | 1.021   | 1.036               | 1.037    | 1.033   |
| Flash, ° F.                        | 525                 | 455      | 500     | 540                 | 470      | 525     | 565                 | 495      | 520     |
| Softening point, ° F.              | 221                 | 218      | 220     | 219                 | 219      | 220     | 221                 | 218      | 222     |
| Pen. 77°/100 g./5"                 | 17                  | 18       | 17      | 15                  | 19       | 18      | 12                  | 12       | 16      |
| Pen. 32°/200 g./60"                | 7                   | 10       | 11      | 9                   | 8        | 8       | 5                   | 6        | 8       |
| Stain                              | 2½                  | 3½       | 4       | 3                   | 3        | 4       | 2                   | 2        | 2½      |

The examples given above should not be considered as limiting this invention to fluxes within the softening point range cited. For other crudes, adjustment in softening point of asphalt bottoms and consistency and flash point of distillate, as well as consistency of the final blended flux, is often required in order to obtain oxidized asphalts exhibiting improved characteristics.

This method of blending and oxidation for the production of oxidized asphalts with improved properties may be extended to include oil fractions, having flash points between 350°-460° F. and asphalts between 150-290° F. softening point, which may in a similar manner be blended to fluxes of suitable consistency or softening point and oxidized to asphalt in the range of 150 to 300° F. softening point.

I claim:

1. An improvement in the manufacture, by oxidation, of coating asphalts which comprises blending 15-70% of 350° to 460° F. flash point oil, such as would be obtained as overhead distillate from a petroleum reduced crude, with 85-30% of 150 to 290° F. softening point asphalt and oxidizing to produce an asphalt having a softening point-penetration relationship of 218° to 222° F.

softening point and 18 to 22 penetration at 77° F./100 grams/5 secs.

2. An improvement in the manufacture, by oxidation, of coating asphalts which comprises blending 15-70% of 350 to 460° F. flash point oil, such as would be obtained as overhead distillate from a petroleum reduced crude, with 85-30% of 150 to 290° F. softening point asphalt and oxidizing to produce a coating asphalt having a softening point-penetration relationship of 218° to 222° F. softening point and 18 to 22 penetration, at 77° F./100 grams/5 secs. and stain of 3½ or less.

3. An improvement in the manufacture by oxidation of coating asphalts which comprises fractionally distilling an asphaltic crude oil to obtain a fraction of 350° to 460° F. flash point oil and a residual 150 to 290° F. softening point asphalt, discarding the intermediate fractions, blending 15% to 70% of the 350° to 460° F. flash point oil with 85% to 30% of the 150° to 290° F. softening point asphalt and oxidizing to produce an asphalt having a softening point-penetration relationship of 218° to 222° F. softening point and 18 to 22 penetration at 77° F./100 grams/5 secs.

KENNETH G. MORRIS.